



US009685267B2

(12) **United States Patent**  
**Matsuura et al.**

(10) **Patent No.:** **US 9,685,267 B2**  
(45) **Date of Patent:** **\*Jun. 20, 2017**

(54) **COIL COMPONENT**(71) Applicant: **TAIYO YUDEN CO., LTD.**, Taito-ku, Tokyo (JP)(72) Inventors: **Hitoshi Matsuura**, Takasaki (JP); **Tomomi Kobayashi**, Takasaki (JP); **Yoshikazu Okino**, Takasaki (JP); **Hidemi Iwao**, Takasaki (JP); **Kenichiro Nogi**, Takasaki (JP); **Kenji Otake**, Takasaki (JP)(73) Assignee: **TAIYO YUDEN CO., LTD.**, Tokyo (JP)

(\* ) Notice: Subject to any disclaimer, the term of this patent is extended or adjusted under 35 U.S.C. 154(b) by 0 days.

This patent is subject to a terminal disclaimer.

(21) Appl. No.: **15/132,102**(22) Filed: **Apr. 18, 2016**(65) **Prior Publication Data**

US 2016/0233019 A1 Aug. 11, 2016

**Related U.S. Application Data**

(63) Continuation of application No. 13/313,982, filed on Dec. 7, 2011, now Pat. No. 9,349,517.

(30) **Foreign Application Priority Data**Jan. 20, 2011 (JP) ..... 2011-009886  
Oct. 24, 2011 (JP) ..... 2011-232371(51) **Int. Cl.****H01F 5/00** (2006.01)  
**H01F 27/28** (2006.01)

(Continued)

(52) **U.S. Cl.**CPC ..... **H01F 27/2823** (2013.01); **H01F 1/047** (2013.01); **H01F 1/08** (2013.01);  
(Continued)(58) **Field of Classification Search**CPC ..... **H01F 1/047**  
(Continued)(56) **References Cited**

## U.S. PATENT DOCUMENTS

2,193,768 A 3/1940 Masumoto et al.  
4,129,444 A 12/1978 Dreyer et al.  
(Continued)

## FOREIGN PATENT DOCUMENTS

CN 1731542 A 2/2006  
CN 101308719 A 11/2008

(Continued)

## OTHER PUBLICATIONS

A Notification of Examination Opinions with Search Report issued by Taiwan Intellectual Property Office, mailed Dec. 19, 2013, for Taiwan counterpart application No. 100140964.

(Continued)

Primary Examiner — Mangtin Lian

Assistant Examiner — Ronald Hinson

(74) Attorney, Agent, or Firm — Law Office of Katsuhiro Arai

(57) **ABSTRACT**

A coil component is of the type where a helical coil is directly contacting a magnetic body where such coil component still meets the demand for electrical current amplification. The coil component is structured in such a way that a helical coil is covered with a magnetic body. The magnetic body is mainly constituted by magnetic alloy grains and contains substantially no glass component, and each of the magnetic alloy grains has an oxide film of the grain on its surface.

**20 Claims, 4 Drawing Sheets**

|                      |           |                 |         |                 |  |  |
|----------------------|-----------|-----------------|---------|-----------------|--|--|
| (51) <b>Int. Cl.</b> |           |                 |         |                 |  |  |
| <i>H01F 17/00</i>    | (2006.01) | 2011/0168939 A1 | 7/2011  | Nakamura et al. |  |  |
| <i>H01F 1/047</i>    | (2006.01) | 2011/0181384 A1 | 7/2011  | Inuduka et al.  |  |  |
| <i>H01F 1/08</i>     | (2006.01) | 2011/0227690 A1 | 9/2011  | Watanabe et al. |  |  |
| <i>H01F 27/255</i>   | (2006.01) | 2011/0267167 A1 | 11/2011 | Ogawa et al.    |  |  |
| <i>H01F 27/29</i>    | (2006.01) | 2012/0038449 A1 | 2/2012  | Ogawa et al.    |  |  |
|                      |           | 2012/0070567 A1 | 3/2012  | Watanabe et al. |  |  |
|                      |           | 2013/0154786 A1 | 6/2013  | Nakajima et al. |  |  |
|                      |           | 2013/0271256 A1 | 10/2013 | Ueno et al.     |  |  |

(52) **U.S. Cl.**

CPC ..... *H01F 17/0033* (2013.01); *H01F 27/255* (2013.01); *H01F 27/2804* (2013.01); *H01F 27/29* (2013.01); *H01F 2027/2809* (2013.01)

(58) **Field of Classification Search**

USPC ..... 336/200

See application file for complete search history.

(56) **References Cited**

## U.S. PATENT DOCUMENTS

|                 |         |                                    |  |  |  |  |
|-----------------|---------|------------------------------------|--|--|--|--|
| 4,921,763 A     | 5/1990  | Karamon                            |  |  |  |  |
| 5,352,522 A     | 10/1994 | Kugimiya et al.                    |  |  |  |  |
| 5,522,946 A     | 6/1996  | Tomita et al.                      |  |  |  |  |
| 5,997,999 A     | 12/1999 | Horiuchi et al.                    |  |  |  |  |
| 6,051,324 A     | 4/2000  | Moorhead et al.                    |  |  |  |  |
| 6,392,525 B1    | 5/2002  | Kato et al.                        |  |  |  |  |
| 6,432,159 B1    | 8/2002  | Saito et al.                       |  |  |  |  |
| 6,515,568 B1    | 2/2003  | Maki et al.                        |  |  |  |  |
| 6,764,643 B2    | 7/2004  | Sagawa et al.                      |  |  |  |  |
| 6,784,782 B2    | 8/2004  | Inoue et al.                       |  |  |  |  |
| 6,814,928 B2    | 11/2004 | Sagawa et al.                      |  |  |  |  |
| 7,422,697 B2    | 9/2008  | Takahashi et al.                   |  |  |  |  |
| 7,446,638 B2    | 11/2008 | Nogi                               |  |  |  |  |
| 7,719,399 B2    | 5/2010  | Iwasaki                            |  |  |  |  |
| 7,843,701 B2    | 11/2010 | Kudo et al.                        |  |  |  |  |
| 8,018,313 B2    | 9/2011  | Tada et al.                        |  |  |  |  |
| 8,416,051 B2    | 4/2013  | Matsuura et al.                    |  |  |  |  |
| 8,427,265 B2    | 4/2013  | Hachiya et al.                     |  |  |  |  |
| 8,866,579 B2    | 10/2014 | Hachiya et al.                     |  |  |  |  |
| 8,896,405 B2    | 11/2014 | Hachiya et al.                     |  |  |  |  |
| 9,349,517 B2 *  | 5/2016  | Matsuura ..... <i>H01F 17/0033</i> |  |  |  |  |
| 2004/0140016 A1 | 7/2004  | Sakamoto et al.                    |  |  |  |  |
| 2004/0209120 A1 | 10/2004 | Inoue et al.                       |  |  |  |  |
| 2005/0199852 A1 | 9/2005  | Takenoshita                        |  |  |  |  |
| 2007/0159282 A1 | 7/2007  | Huang et al.                       |  |  |  |  |
| 2007/0290161 A1 | 12/2007 | Tokuoka et al.                     |  |  |  |  |
| 2008/0003126 A1 | 1/2008  | Watanabe et al.                    |  |  |  |  |
| 2008/0012679 A1 | 1/2008  | Okabe et al.                       |  |  |  |  |
| 2008/0029300 A1 | 2/2008  | Harada et al.                      |  |  |  |  |
| 2008/0061264 A1 | 3/2008  | Maeda et al.                       |  |  |  |  |
| 2008/0152897 A1 | 6/2008  | Maeda et al.                       |  |  |  |  |
| 2008/0231409 A1 | 9/2008  | Kugai et al.                       |  |  |  |  |
| 2008/0278273 A1 | 11/2008 | Lee et al.                         |  |  |  |  |
| 2009/0003191 A1 | 1/2009  | Inuzuka et al.                     |  |  |  |  |
| 2009/0045905 A1 | 2/2009  | Nakagawa et al.                    |  |  |  |  |
| 2009/0102589 A1 | 4/2009  | Lee et al.                         |  |  |  |  |
| 2009/0140833 A1 | 6/2009  | Tan et al.                         |  |  |  |  |
| 2010/0033286 A1 | 2/2010  | Katayama et al.                    |  |  |  |  |
| 2010/0253463 A1 | 10/2010 | Shimomura et al.                   |  |  |  |  |
| 2010/0287764 A1 | 11/2010 | McGregor et al.                    |  |  |  |  |
| 2010/0289609 A1 | 11/2010 | Liao et al.                        |  |  |  |  |
| 2011/0024670 A1 | 2/2011  | Otsuki et al.                      |  |  |  |  |
| 2011/0024671 A1 | 2/2011  | Otsuki et al.                      |  |  |  |  |
| 2011/0133881 A1 | 6/2011  | Nakajima et al.                    |  |  |  |  |

## FOREIGN PATENT DOCUMENTS

|    |               |         |
|----|---------------|---------|
| CN | 101927344 A   | 12/2010 |
| CN | 102007549 A   | 4/2011  |
| JP | H04346204 A   | 12/1992 |
| JP | 07201570 A    | 8/1995  |
| JP | H09074011 A   | 3/1997  |
| JP | 2000030925 A  | 1/2000  |
| JP | 2001011563 A  | 1/2001  |
| JP | 2001118725 A  | 4/2001  |
| JP | 2002305108 A  | 10/2002 |
| JP | 2002313620 A  | 10/2002 |
| JP | 2002343618 A  | 11/2002 |
| JP | 2005150257 A  | 6/2005  |
| JP | 2005286145 A  | 10/2005 |
| JP | 2006179621 A  | 7/2006  |
| JP | 2007019134 A  | 1/2007  |
| JP | 2007027354 A  | 2/2007  |
| JP | 2007123703 A  | 5/2007  |
| JP | 2007258427 A  | 10/2007 |
| JP | 2007299871 A  | 11/2007 |
| JP | 2008028162 A  | 2/2008  |
| JP | 2008041961 A  | 2/2008  |
| JP | 2008195986 A  | 8/2008  |
| JP | 2009088496 A  | 4/2009  |
| JP | 2009088502 A  | 4/2009  |
| TW | 200845057 A   | 11/2008 |
| TW | M388724 U1    | 9/2010  |
| WO | 2009128425 A1 | 10/2009 |
| WO | 2010113681 A1 | 10/2010 |
| WO | 2011001958 A1 | 1/2011  |

## OTHER PUBLICATIONS

A Notification of First Chinese Office Action with Search Report issued by the State Intellectual Property Office of China, issued on Nov. 26, 2013, for Chinese counterpart application No. 201210005436.0.

Final Office Action issued by U.S. Patent and Trademark Office, dated Aug. 1, 2014, for related U.S. Appl. No. 13/313,982.

Final Office Action issued by U.S. Patent and Trademark Office, dated Jul. 15, 2015, for related U.S. Appl. No. 13/313,982.

Final Office Action issued by U.S. Patent and Trademark Office, dated Sep. 18, 2013, for related U.S. Appl. No. 13/313,982.

Non-Final Office Action issued by U.S. Patent and Trademark Office, dated Dec. 23, 2014, for related U.S. Appl. No. 13/313,982.

Non-Final Office Action issued by U.S. Patent and Trademark Office, dated Jan. 2, 2014, for related U.S. Appl. No. 13/313,982.

Non-Final Office Action issued by U.S. Patent and Trademark Office, dated Mar. 5, 2013, for related U.S. Appl. No. 13/313,982.

Notice of Allowance issued by U.S. Patent and Trademark Office, dated Jan. 20, 2016, for related U.S. Appl. No. 13/313,982.

\* cited by examiner

Fig. 1



Fig. 2



Fig. 3



Fig. 4



Fig. 5



Fig. 6



Fig. 7



# 1

## COIL COMPONENT

### CROSS-REFERENCE TO RELATED APPLICATIONS

This application is a continuation of U.S. patent application Ser. No. 13/313,982, filed Dec. 7, 2011, which claims priority to Japanese Patent Application No. 2011-009886, filed Jan. 20, 2011, and No. 2011-232371, filed Oct. 24, 2011, each disclosure of which is herein incorporated by reference in its entirety. The applicant(s) herein explicitly rescind(s) and retract(s) any prior disclaimers or disavowals made in any parent, child or related prosecution history with regard to any subject matter supported by the present application.

### BACKGROUND

#### Field of the Invention

The present invention relates to a coil component structured in such a way that a helical coil is covered with a magnetic body.

#### Description of the Related Art

Coil components (so-called “inductance components”), representative examples of which are inductors, choke coils and transformers, are structured in such a way that a helical coil is covered with a magnetic body. For the magnetic body covering the coil, Ni—Cu—Zn ferrite and other ferrites (=ceramics whose main constituent is iron oxide) are generally used.

In recent years, there has been a demand for coil components of this type offering electrical current amplification (=higher rated current) and, to meet this need, switching the material for the magnetic body from conventional ferrites to Fe—Cr—Si alloy is being examined (refer to patent Literature 1).

This Fe—Cr—Si alloy has a higher saturated magnetic flux density than conventional ferrites, but its volume resistivity is much lower than conventional ferrites. In other words, to switch the material for magnetic body from conventional ferrites to Fe—Cr—Si alloy for a coil component of the type where the helical coil is directly contacting the magnetic body, such as a coil component of the laminated type or the powder-compact type, an ingenious idea is needed to bring the volume resistivity of the magnetic body itself, which is constituted by Fe—Cr—Si alloy grains, closer to the volume resistivity of the magnetic body constituted by ferrite grains, or preferably increase the volume resistivity of the former beyond that of the latter.

In essence, without ensuring a high volume resistivity of the magnetic body itself which is constituted by Fe—Cr—Si alloy grains, the saturated magnetic flux density of the material cannot be utilized to increase the saturated magnetic flux density of the component and, due to the phenomenon of current leaking from the coil to the magnetic body and disturbing the magnetic field, the inductance of the component itself will drop.

Note that Patent Literature 1 mentioned above discloses a method for manufacturing a magnetic body for coil component of the laminated type, which comprises laminating a magnetic body layer formed by a magnetic paste containing Fe—Cr—Si alloy grains as well as a glass component, with a conductor pattern, baking the laminate in a nitrogen ambience (=reducing ambience), and then impregnating the baked laminate with a thermo-setting resin.

However, this manufacturing method allows the glass component in the magnetic paste to remain in the magnetic

# 2

body, and this glass component in the magnetic body reduces the volume ratio of Fe—Cr—Si alloy grains, which in turn lowers the saturated magnetic flux density of the component itself.

Any discussion of problems and solutions involved in the related art has been included in this disclosure solely for the purposes of providing a context for the present invention, and should not be taken as an admission that any or all of the discussion were known at the time the invention was made.

### BACKGROUND ART LITERATURES

[Patent Literature 1] Japanese Patent Laid-open No. 2007-027354

### SUMMARY

An object of the present invention is to provide a coil component of the type where a helical coil is directly contacting a magnetic body, where such coil component still meets the demand for electrical current amplification.

To achieve the aforementioned object, the present invention provides a coil component of the type where a helical coil covered with a magnetic body is directly contacting the magnetic body, wherein the aforementioned magnetic body is mainly constituted by magnetic alloy grains and substantially free of a glass component, and the aforementioned magnetic alloy grains have an oxide film of magnetic alloy grains on their surface.

In some embodiments, the term “oxide film” refers to a film formed by oxidization of magnetic alloy grains after being shaped into the magnetic body or the coil component, said film being substantially the sole film formed on the magnetic alloy grains in the magnetic body. In some embodiments, the term “directly contacting” refers to physically contacting without any additional intervening layers therebetween. In some embodiments, the term “mainly constituted by” refers to being materially constituted by, being characterized by, or being constituted by, as the main component. In some embodiments, the term “substantially free” refers to being free to a degree equivalent to zero, being materially free, containing less than 5% or less than 1%, or containing less than a detectable degree. In some embodiments, the magnetic alloy grains are bonded to each other mostly via the oxide film and partially directly without the oxide film. In some embodiments, the magnetic alloy grains adjacent to the coil are bonded to the coil via the oxide film without any additional intervening layers therebetween. In this disclosure, any defined meanings do not necessarily exclude ordinary and customary meanings in some embodiments. Also, in this disclosure, “the invention” or “the present invention” refers to at least one of the embodiments or aspects explicitly, necessarily, or inherently disclosed herein. Further, in this disclosure, “a” may refer to a species or a genus including multiple species. The term “magnetic alloy grains” refers to magnetic alloy grains including an oxide film formed thereon, but also refers to magnetic alloy grains without an oxide film, depending on the context.

According to the present invention, magnetic alloy grains constituting the magnetic body have an oxide film (=insulation film) of magnetic alloy grains on their surface, and magnetic alloy grains in the magnetic body directly bind with one another via the oxide film that serves as an insulation film, and also magnetic alloy grains near the coil adhere to the coil via the oxide film that serves as an insulation film, and for these reasons a high volume resistivity of the magnetic body mainly constituted by magnetic

alloy grains can be ensured. In addition, since the magnetic body does not contain a glass component, the volume ratio of magnetic alloy grains does not drop unlike when there is a glass component in the magnetic body, which prevents the saturated magnetic flux density of the component itself from dropping due to a lower volume ratio.

In other words, although the coil component is of the type where the coil is directly contacting the magnetic body, the saturated magnetic flux density of the component itself can be increased by effectively utilizing the saturated magnetic flux density of the magnetic alloy material, which helps meet the demand for electrical current amplification and also prevents the phenomenon of current leaking from the coil to the magnetic body and disturbing the magnetic field, which in turn prevents the inductance of the component itself from dropping.

The aforementioned object and other objects, constitution/characteristics and operation/effects of the present invention are made clear by the following explanations and attached drawings.

#### BRIEF DESCRIPTION OF THE DRAWINGS

These and other features of this invention will now be described with reference to the drawings of preferred embodiments which are intended to illustrate and not to limit the invention. The drawings are greatly simplified for illustrative purposes and are not necessarily to scale.

FIG. 1 is an external perspective view of a coil component of the laminated type.

FIG. 2 is an enlarged sectional view taken along line S11-S11 in FIG. 1.

FIG. 3 is an exploded view of the component shown in FIG. 1.

FIG. 4 is a graph showing the granularity distribution of grains constituting the magnetic body shown in FIG. 2.

FIG. 5 is a schematic view showing the condition of grains according to an image obtained by observing the magnetic body in FIG. 2 with a transmission electron microscope.

FIG. 6 is a schematic view showing the condition of grains according to an image obtained by observing the magnetic body before the binder removal process with a transmission electron microscope.

FIG. 7 is a schematic view showing the condition of grains according to an image obtained by observing the magnetic body after the binder removal process with a transmission electron microscope.

#### DESCRIPTION OF THE SYMBOLS

- 1 Magnetic alloy grain
- 2 Oxide film
- 3 Pore
- 4 Mixture of solvent and binder
- 10 Coil component
- 11 Main component body
- 12 Magnetic body
- 13 Coil
- 14, 15 External terminal

#### DETAILED DESCRIPTION OF EMBODIMENTS

##### [Example of Specific Structure of Coil Component]

First, an example of specific structure where the present invention is applied to a coil component of the laminated type is explained by referring to FIGS. 1 to 5.

A coil component 10 shown in FIG. 1 has a rectangular solid shape of approx. 3.2 mm in length L, approx. 1.6 mm in width W, and approx. 0.8 mm in height H. This coil component 10 has a main component body 11 of rectangular solid shape and a pair of external terminals 14, 15 provided at both ends in the length direction of the main component body 11. As shown in FIG. 2, the main component body 11 has a magnetic body 12 of rectangular solid shape and a helical coil 13 covered with the magnetic body 12, where one end of the coil 13 is connected to the external terminal 14, while the other end is connected to the external terminal 15.

As shown in FIG. 3, the magnetic body 12 is structured in such a way that a total of 20 layers of magnetic layers ML1 to ML6 are put together and it has a length of approx. 3.2 mm, width of approx. 1.6 mm, and thickness (height) of approx. 0.8 mm. The length, width and thickness of each of the magnetic layers ML1 to ML6 are approx. 3.2 mm, approx. 1.6 mm and approx. 40 respectively. This magnetic body 12 is mainly constituted by Fe—Cr—Si alloy grains and does not contain a glass component. The composition of the Fe—Cr—Si alloy grains is 88 to 96.5 percent by weight of Fe, 2 to 8 percent by weight of Cr, and 1.5 to 7 percent by weight of Si.

As shown in FIG. 4, Fe—Cr—Si alloy grains constituting the magnetic body 12 have a d50 (median diameter) of 10  $\mu\text{m}$ , d10 of 3  $\mu\text{m}$  and d90 of 16  $\mu\text{m}$  when their grain size is considered based on volume, where d10/d50 is 0.3 and d90/d50 is 1.6. Also as shown in FIG. 5, an oxide film (=insulation film) 2 of Fe—Cr—Si alloy grains is present on the surface of each Fe—Cr—Si alloy grain 1, and Fe—Cr—Si alloy grains 1 in the magnetic body 12 bind with one another via the oxide film 2 that serves as an insulation film, while Fe—Cr—Si alloy grains 1 near the coil 13 adhere to the coil 13 via the oxide film 2 that serves as an insulation film. This oxide film 2 has been confirmed to contain at least the magnetic substance  $\text{Fe}_3\text{O}_4$  and non-magnetic substances  $\text{Fe}_2\text{O}_3$  and  $\text{Cr}_2\text{O}_3$ .

It should be noted that FIG. 4 shows a granularity distribution measured with a grain-size/granularity-distribution measuring apparatus utilizing the laser diffraction scattering method (Microtrack manufactured by Nikkiso Co., Ltd.). FIG. 5 shows a schematic view of the condition of grains according to an image obtained by observing the magnetic body 12 with a transmission electron microscope. Fe—Cr—Si alloy grains 1 constituting the magnetic body 12 are not actually perfect spheres, but all grains here are depicted as spheres in order to illustrate that their grain sizes have a distribution. Also, while the thickness of the oxide film 2 present on the surface of each grain actually varies over a range of 0.05 to 0.2  $\mu\text{m}$ , the oxide film 2 here is depicted as having a uniform thickness throughout in order to illustrate that the oxide film 2 is present on the grain surface.

As shown in FIG. 3, the coil 13 is structured in such a way that a total of five coil segments CS1 to CS5, and a total of four relay segments IS1 to IS4 connecting the coil segments CS1 to CS5, are put together in a helical pattern and the number of windings is approx. 3.5. This coil 13 is mainly constituted by Ag grains. When their grain size is considered based on volume, Ag grains have a d50 (median diameter) of 5  $\mu\text{m}$ .

The four coil segments CS1 to CS4 have a C shape, while one coil segment CS5 has a thin strip shape. Each of the coil segments CS1 to CS5 has a thickness of approx. 20  $\mu\text{m}$  and width of approx. 0.2 mm. The top coil segment CS1 has an L-shaped leader part LS1 which is continuously formed with

the coil segment and utilized to connect to external terminal **14**, while the bottom coil segment **CS5** also has an L-shaped leader part **LS2** which is continuously formed with the coil segment and utilized to connect to external terminal **15**. Each of the relay segments **IS1** to **IS4** has a column shape that passes through the corresponding magnetic layer **ML1**, **ML2**, **ML3** or **ML4**, where each segment has a bore of approx. 15  $\mu\text{m}$ .

As shown in FIGS. 1 and 2, the external terminals **14**, **15** cover each end face, in the length direction, of the main component body **11** as well as four side faces near the end face, and have a thickness of approx. 20  $\mu\text{m}$ . The one external terminal **14** connects to the edge of the leader part **LS1** of the top coil segment **CS1**, while the other external terminal **15** connects to the edge of the leader part **LS2** of the bottom coil segment **CS5**. These external terminals **14**, **15** are mainly constituted by Ag grains. When their grain size is considered based on volume, Ag grains have a  $d_{50}$  (median diameter) of 5  $\mu\text{m}$ .

[Example of Specific Method for Manufacturing Coil Component]

Next, an example of a specific method for manufacturing the aforementioned coil component **10** is explained by referring to FIGS. 3, 5, 6 and 7.

When manufacturing the aforementioned coil component **10**, a doctor blade, die coater, or other coating machine (not illustrated) is used to coat a prepared magnetic paste onto the surface of a plastic base film (not illustrated), after which the coated base film is dried at approx. 80° C. for approx. 5 minutes using a hot-air dryer or other dryer (not illustrated), to create first to sixth sheets that correspond to the magnetic layers **ML1** to **ML6** (refer to FIG. 3), respectively, and have a size appropriate for multiple-part processing.

The composition of the magnetic paste used here is 85 percent by weight of Fe—Cr—Si alloy grains, 13 percent by weight of butyl carbitol (solvent) and 2 percent by weight of polyvinyl butyral (binder), where Fe—Cr—Si alloy grains have the  $d_{50}$  (median diameter),  $d_{10}$  and  $d_{90}$  as mentioned earlier.

Next, a stamping machine, laser processing machine, or other piercing machine (not illustrated) is used to pierce the first sheet corresponding to the magnetic layer **ML1** (refer to FIG. 3), to form through holes corresponding to the relay segment **IS1** (refer to FIG. 3) in a specified layout. Similarly, the second to fourth sheets corresponding to the magnetic layers **ML2** to **ML4** (refer to FIG. 3) are pierced to form through holes corresponding to the relay segments **IS2** to **IS4** (refer to FIG. 3) in specified layouts.

Next, a screen printer, gravure printer or other printer (not illustrated) is used to print a prepared conductive paste onto the surface of the first sheet corresponding to the magnetic layer **ML1** (refer to FIG. 3), after which the printed sheet is dried at approx. 80° C. for approx. 5 minutes using a hot-air dryer or other dryer (not illustrated), to create a first printed layer corresponding to the coil segment **CS1** (refer to FIG. 3) in a specified layout. Similarly, second to fifth printed layers corresponding to the coil segments **CS2** to **CS5** (refer to FIG. 3) are created in specified layouts on the surfaces of the second to fifth sheets corresponding to the magnetic layers **ML2** to **ML5** (refer to FIG. 3).

The composition of the conductive paste used here is 85 percent by weight of Ag grains, 13 percent by weight of butyl carbitol (solvent) and 2 percent by weight of polyvinyl butyral (binder), where Ag grains have the  $d_{50}$  (median diameter) as mentioned earlier.

The through holes formed in specified layouts in the first to fourth sheets corresponding to the magnetic layers **ML1**

to **ML4** (refer to FIG. 3) are positioned in a manner overlapping with the edges of the first to fourth printed layers in specified layouts, respectively, so that part of the conductive paste is filled in each through hole when the first to fourth printed layers are created, to form first to fourth filled parts corresponding to the relay segments **IS1** to **IS4** (refer to FIG. 3).

Next, a suction transfer machine and press machine (both not illustrated) are used to stack in the order shown in FIG. 10 **3** and thermally compress the first to fourth sheets (corresponding to the magnetic layers **ML1** to **ML4**) each having a printed layer and filled part, the fifth sheet (corresponding to the magnetic layer **ML5**) having only a printed layer, and the sixth sheet (corresponding to the magnetic layer **ML6**) having neither a printed layer nor filled part, to create a laminate.

Next, a dicing machine, laser processing machine, or other cutting machine (not illustrated) is used to cut the laminate to the size of the main component body to create a 20 chip before heat treatment (including a magnetic body and coil before heat treatment).

Next, a baking furnace or other heat treatment machine (not illustrated) is used to heat-treat multiple chips before heat treatment in batch in an atmosphere or other oxidizing ambience. This heat treatment includes a binder removal process and an oxide film forming process, where the binder removal process is implemented under conditions of approx. 300° C. for approx. 1 hour, while the oxide film forming process is implemented under conditions of approx. 750° C. and approx. 2 hours.

As shown in FIG. 6, before the binder removal process, the chip before heat treatment has many fine voids between Fe—Cr—Si alloy grains **1** in the magnetic body before heat treatment and, while these fine voids are filled with a mixture **4** of solvent and binder, this mixture is lost in the binder removal process and therefore by the time the binder removal process is completed, these fine voids have changed to pores **3**, as shown in FIG. 7. Also, while many fine voids are present between Ag grains in the coil before heat treatment and these fine voids are filled with a mixture of solvent and binder, this mixture is lost in the binder removal process.

In the oxide film forming process after the binder removal process, Fe—Cr—Si alloy grains **1** in the magnetic body before heat treatment gather closely to create the magnetic body **12** (refer to FIGS. 1 and 2), as shown in FIG. 5, while at the same time the oxide film **2** of Fe—Cr—Si alloy grains **1** is formed on the surface of each grain **1**. Also, Ag grains in the coil before heat treatment are sintered to create the coil 40 **13** (refer to FIGS. 1 and 2), thereby creating the main component body **11** (refer to FIGS. 1 and 2).

FIGS. 6 and 7 provide schematic views of the condition of grains according to images obtained by observing the magnetic bodies before and after the binder removal process 45 with a transmission electron microscope. Fe—Cr—Si alloy grains **1** constituting the magnetic body before heat treatment are actually not perfect spheres, but all grains here are depicted as spheres to maintain consistency with FIG. 5.

Next, a dip coater, roller coater, or other coater (not 60 illustrated) is used to coat a prepared conductive paste onto both ends in the length direction of the main component body **11**, and then the coated main component body is baked in a baking furnace or other heat treatment machine (not illustrated) under conditions of approx. 600° C. for approx. 65 1 hour to remove the solvent and binder in the baking process, while also sintering the Ag grains, to create the external terminals **14**, **15** (refer to FIGS. 1 and 2).

The composition of the conductive paste used here is 85 percent by weight of Ag grains, 13 percent by weight of butyl carbitol (solvent) and 2 percent by weight of polyvinyl butyral (binder), where Ag grains have the d50 (median diameter) as mentioned earlier.

[Effects]

Next, the effects of the aforementioned coil component 10 are explained by referring to Sample No. 4 in Table 1.

TABLE 1

| Sample | d50<br>( $\mu\text{m}$ ) | d10<br>( $\mu\text{m}$ ) | d90<br>( $\mu\text{m}$ ) | d10/<br>d50 | d90/<br>d50 | Volume<br>resistivity<br>( $\Omega \cdot \text{cm}$ ) | $L \times$<br>Idc1<br>( $\mu\text{H} \cdot$<br>A) |
|--------|--------------------------|--------------------------|--------------------------|-------------|-------------|-------------------------------------------------------|---------------------------------------------------|
| No. 1  | 10                       | 0.5                      | 16                       | 0.05        | 1.6         | $1.1 \times 10^9$                                     | ○ X                                               |
| No. 2  | 10                       | 1                        | 16                       | 0.1         | 1.6         | $9.5 \times 10^8$                                     | ○ 6.5 ○                                           |
| No. 3  | 10                       | 2                        | 16                       | 0.2         | 1.6         | $6.0 \times 10^8$                                     | ○ 7.2 ○                                           |
| No. 4  | 10                       | 3                        | 16                       | 0.3         | 1.6         | $5.2 \times 10^8$                                     | ○ 8.3 ○                                           |
| No. 5  | 10                       | 4                        | 16                       | 0.4         | 1.6         | $4.1 \times 10^8$                                     | ○ 8.3 ○                                           |
| No. 6  | 10                       | 5                        | 16                       | 0.5         | 1.6         | $9.0 \times 10^7$                                     | ○ 8.4 ○                                           |
| No. 7  | 10                       | 6                        | 16                       | 0.6         | 1.6         | $5.6 \times 10^7$                                     | ○ 8.4 ○                                           |
| No. 8  | 10                       | 7                        | 16                       | 0.7         | 1.6         | $2.1 \times 10^7$                                     | ○ 8.4 ○                                           |
| No. 9  | 10                       | 8                        | 16                       | 0.8         | 1.6         | $8.5 \times 10^6$                                     | X 8.5 ○                                           |
| No. 10 | 10                       | 9                        | 16                       | 0.9         | 1.6         | $3.1 \times 10^6$                                     | X 8.5 ○                                           |
| No. 11 | 10                       | 3                        | 13                       | 0.3         | 1.3         | $1.0 \times 10^9$                                     | ○ 5.0 ○                                           |
| No. 12 | 10                       | 3                        | 14                       | 0.3         | 1.4         | $9.5 \times 10^8$                                     | ○ 5.8 ○                                           |
| No. 13 | 10                       | 3                        | 15                       | 0.3         | 1.5         | $7.3 \times 10^8$                                     | ○ 7.2 ○                                           |
| No. 4  | 10                       | 3                        | 16                       | 0.3         | 1.6         | $5.2 \times 10^8$                                     | ○ 8.3 ○                                           |
| No. 14 | 10                       | 3                        | 17                       | 0.3         | 1.7         | $3.7 \times 10^8$                                     | ○ 8.3 ○                                           |
| No. 15 | 10                       | 3                        | 18                       | 0.3         | 1.8         | $2.0 \times 10^8$                                     | ○ 8.3 ○                                           |
| No. 16 | 10                       | 3                        | 19                       | 0.3         | 1.9         | $1.0 \times 10^8$                                     | ○ 8.3 ○                                           |
| No. 17 | 10                       | 3                        | 20                       | 0.3         | 2.0         | $8.7 \times 10^7$                                     | ○ 8.3 ○                                           |
| No. 18 | 10                       | 3                        | 30                       | 0.3         | 3.0         | $4.6 \times 10^7$                                     | ○ 8.4 ○                                           |
| No. 19 | 10                       | 3                        | 40                       | 0.3         | 4.0         | $2.6 \times 10^7$                                     | ○ 8.4 ○                                           |
| No. 20 | 10                       | 3                        | 50                       | 0.3         | 5.0         | $1.1 \times 10^7$                                     | ○ 8.5 ○                                           |
| No. 21 | 10                       | 3                        | 55                       | 0.3         | 5.5         | $7.0 \times 10^6$                                     | X 8.5 ○                                           |
| No. 22 | 10                       | 3                        | 60                       | 0.3         | 6.0         | $4.2 \times 10^6$                                     | X 8.6 ○                                           |

With the aforementioned coil component 10, Fe—Cr—Si alloy grains constituting the magnetic body 12 each have an oxide film (=insulation film) of Fe—Cr—Si alloy grains on the surface, and Fe—Cr—Si alloy grains in the magnetic body 12 bind with one another via the oxide film that serves as an insulation film, while Fe—Cr—Si alloy grains near the coil 13 adhere to the coil 13 via the oxide film that serves as an insulation film, and therefore a high volume resistivity can be ensured for the magnetic body itself which is mainly constituted by Fe—Cr—Si alloy grains. Also, the magnetic body 12 does not contain a glass component, so the volume ratio of Fe—Cr—Si alloy grains does not drop, unlike when there is a glass component in the magnetic body 12, which prevents the saturated magnetic flux density of the component itself from dropping due to a lower volume ratio.

In other words, although the coil component is of the type where the coil 13 is directly contacting the magnetic body 12, the saturated magnetic flux density of the component itself can be increased by effectively utilizing the saturated magnetic flux density of the Fe—Cr—Si alloy material, which helps meet the demand for electrical current amplification and also prevents the phenomenon of current leaking from the coil 13 to the magnetic body 12 and disturbing the magnetic field, which in turn prevents the inductance of the component itself from dropping.

This effect can also be demonstrated by the volume resistivity and  $L \times \text{Idc1}$  of Sample No. 4 in Table 1 that corresponds to the aforementioned coil component 10. Each volume resistivity ( $\Omega \cdot \text{cm}$ ) shown in Table 1 indicates the volume resistivity of the magnetic body 12 itself, measured with a commercial LCR meter. On the other hand, each  $L \times \text{Idc1}$  ( $\mu\text{H} \cdot \text{A}$ ) shown in Table 1 indicates the product of the

initial inductance ( $L$ ) and the direct-current bias current ( $\text{Idc1}$ ) when the initial inductance ( $L$ ) has dropped by 20%, measured at a measurement frequency of 100 kHz using a commercial LCR meter.

Now, the acceptance judgment criteria for volume resistivity and  $L \times \text{Idc1}$  are explained. Given the fact that conventional coil components generally use Ni—Cu—Zn ferrite, among other ferrites, for their magnetic body, a coil component was created based on the same structure and 10 using the same manufacturing method as those used by the aforementioned coil component 10, except that “Ni—Cu—Zn ferrite grains with a d50 (median diameter) of 10  $\mu\text{m}$ , when their grain size is considered based on volume, were used instead of Fe—Cr—Si alloy grains” and that “a baking process was adopted under conditions of approx. 900° C. for approx. 2 hours, instead of the oxide film forming process” (the obtained coil component is hereinafter referred to as the “comparative coil component”).

When the volume resistivity and  $L \times \text{Idc1}$  of the magnetic body of this comparative coil component were measured in the same manners as mentioned above, the volume resistivity was  $5.0 \times 10^6 \Omega \cdot \text{cm}$ , while  $L \times \text{Idc1}$  was  $5.2 \mu\text{H} \cdot \text{A}$ . With conventional coil components using Ni—Cu—Zn ferrite grains, however, the volume resistivity of the magnetic body is increased to  $1.0 \times 10^7 \Omega \cdot \text{cm}$  or higher by manipulating the grain composition, impregnating it with resin, or using other methods, and accordingly the acceptance judgment criterion for volume resistivity was set to “ $1.0 \times 10^7 \Omega \cdot \text{cm}$ ”; i.e., values equal to or higher than this criterion value were judged 20 “acceptable (○),” while those lower than the criterion value were judged “unacceptable (X).” Meanwhile, the acceptance judgment criterion for  $L \times \text{Idc1}$  was set to the measured value of  $L \times \text{Idc1}$  of the comparative coil component, or specifically “ $5.2 \mu\text{H} \cdot \text{A}$ ;” i.e., values higher than this criterion value were 30 judged “acceptable (○),” while those equal to or lower than the criterion value were judged “unacceptable.”

As evident from the volume resistivity and  $L \times \text{Idc1}$  of Sample No. 4, the volume resistivity of Sample No. 4 corresponding to the aforementioned coil component 10 is 40  $5.2 \times 10^8 \Omega \cdot \text{cm}$ , which is higher than the aforementioned acceptance judgment criterion for volume resistivity ( $1.0 \times 10^7 \Omega \cdot \text{cm}$ ), while  $L \times \text{Idc1}$  of Sample No. 4 corresponding to the aforementioned coil component 10 is  $8.3 \mu\text{H} \cdot \text{A}$ , which is higher than the aforementioned acceptance judgment criterion for  $L \times \text{Idc1}$  ( $5.2 \mu\text{H} \cdot \text{A}$ ), and therefore these values demonstrate the aforementioned effects.

[Verification of Optimal Granularity Distribution]

Next, the result of verification of an optimal granularity distribution ( $d10/d50$  and  $d90/d50$ ) of Fe—Cr—Si alloy grains constituting the magnetic body 12 of the aforementioned coil component 10 (Sample No. 4) is explained by referring to Table 1.

With the aforementioned coil component 10 (Sample No. 4), the Fe—Cr—Si alloy grains used to constitute the 55 magnetic body 12 had a d50 (median diameter) of 10  $\mu\text{m}$ , d10 of 3  $\mu\text{m}$  and d90 of 16  $\mu\text{m}$  when their grain size was considered based on volume. Whether or not effects similar to those explained above could be obtained using grains of a different granularity distribution ( $d10/d50$  and  $d90/d50$ ) was evaluated.

Sample Nos. 1 to 3 and 5 to 10 shown in Table 1 are coil components having the same structure and made by the same manufacturing method as those used by the aforementioned coil component 10, except that “Fe—Cr—Si alloy grains having a different d10 value from that of the aforementioned coil component 10 (Sample No. 4) were used.” Also, Sample Nos. 11 to 22 shown in Table 1 are coil

components having the same structure and made by the same manufacturing method as those used by the aforementioned coil component **10** (Sample No. 4), except that “Fe—Cr—Si alloy grains having a different d90 value from that of the aforementioned coil component **10** (Sample No. 4) were used.”

As evident from the volume resistivity and  $L \times I_{dc1}$  values of Sample Nos. 1 to 10, a volume resistivity higher than the aforementioned acceptance judgment criterion for volume resistivity ( $1.0 \times 10^7 \Omega \cdot \text{cm}$ ) can be obtained as long as  $d10$  is 7  $\mu\text{m}$  or less, while a  $L \times I_{dc1}$  higher than the aforementioned acceptance judgment criterion for  $L \times I_{dc1}$  ( $5.2 \mu\text{H} \cdot \text{A}$ ) can be obtained as long as  $d10$  is 1  $\mu\text{m}$  or more. In other words, excellent volume resistivity and  $L \times I_{dc1}$  can be obtained as long as  $d10$  is in a range of 1 to 7.0  $\mu\text{m}$  ( $d10/d50$  is in a range of 0.1 to 0.7).

Also, as is evident from the volume resistivity and  $L \times I_{dc1}$  values of Sample Nos. 11 to 22, a volume resistivity higher than the aforementioned acceptance judgment criterion for volume resistivity ( $1.0 \times 10^7 \Omega \cdot \text{cm}$ ) can be obtained as long as  $d90$  is 50  $\mu\text{m}$  or less, while a  $L \times I_{dc1}$  higher than the aforementioned acceptance judgment criterion for  $L \times I_{dc1}$  ( $5.2 \mu\text{H} \cdot \text{A}$ ) can be obtained as long as  $d90$  is 14  $\mu\text{m}$  or more. In other words, excellent volume resistivity and  $L \times I_{dc1}$  can be obtained as long as  $d90$  is in a range of 14 to 50  $\mu\text{m}$  ( $d90/d50$  is in a range of 1.4 to 5.0).

In essence, the above confirms that, as long as  $d10/d50$ , when the grain size is considered based on volume, is in a range of 0.1 to 0.7 and  $d90/d50$  is in a range of 1.4 to 5.0, Fe—Cr—Si alloy grains whose granularity distribution ( $d10/d50$  and  $d90/d50$ ) is different can be used to achieve the same effects as mentioned above.

#### [Verification of Optimal Median Diameter]

Next, the result of verification of optimal median diameter ( $d50$ ) of Fe—Cr—Si alloy grains constituting the magnetic body **12** of the aforementioned coil component **10** (Sample No. 4) is explained by referring to Table 2.

TABLE 2

| Sample | $d50$<br>( $\mu\text{m}$ ) | $d10$<br>( $\mu\text{m}$ ) | $d90$<br>( $\mu\text{m}$ ) | $d10/d50$ | $d90/d50$ | Volume<br>resistivity<br>( $\Omega \cdot \text{cm}$ ) | $L \times$<br>$I_{dc1}$<br>( $\mu\text{H} \cdot$<br>$\text{A}$ ) |
|--------|----------------------------|----------------------------|----------------------------|-----------|-----------|-------------------------------------------------------|------------------------------------------------------------------|
| No. 23 | 1                          | 0.3                        | 1.6                        | 0.3       | 1.6       | $4.1 \times 10^{10}$                                  | ○ 3.4 X                                                          |
| No. 24 | 2                          | 0.6                        | 3.2                        | 0.3       | 1.6       | $9.3 \times 10^9$                                     | ○ 5.0 X                                                          |
| No. 25 | 3                          | 0.9                        | 4.8                        | 0.3       | 1.6       | $5.1 \times 10^9$                                     | ○ 7.2 ○                                                          |
| No. 26 | 4                          | 1.2                        | 6.4                        | 0.3       | 1.6       | $2.2 \times 10^9$                                     | ○ 7.5 ○                                                          |
| No. 27 | 5                          | 1.5                        | 8                          | 0.3       | 1.6       | $9.2 \times 10^8$                                     | ○ 7.7 ○                                                          |
| No. 4  | 10                         | 3                          | 16                         | 0.3       | 1.6       | $5.2 \times 10^8$                                     | ○ 8.3 ○                                                          |
| No. 28 | 15                         | 4.5                        | 24                         | 0.3       | 1.6       | $9.6 \times 10^7$                                     | ○ 8.4 ○                                                          |
| No. 29 | 20                         | 6                          | 32                         | 0.3       | 1.6       | $1.1 \times 10^7$                                     | ○ 8.6 ○                                                          |
| No. 30 | 21                         | 6.3                        | 33.6                       | 0.3       | 1.6       | $9.5 \times 10^6$                                     | X 8.7 ○                                                          |
| No. 31 | 22                         | 6.6                        | 35.2                       | 0.3       | 1.6       | $8.7 \times 10^6$                                     | X 8.7 ○                                                          |

With the aforementioned coil component **10** (Sample No. 4), the Fe—Cr—Si alloy grains used to constitute the magnetic body **12** had a  $d50$  (median diameter) of 10  $\mu\text{m}$ ,  $d10$  of 3  $\mu\text{m}$  and  $d90$  of 16  $\mu\text{m}$  when their grain size was considered based on volume. Whether or not effects similar to those explained above could be obtained using grains of a different  $d50$  (median diameter) was checked.

Sample Nos. 23 to 31 shown in Table 2 are coil components having the same structure and made by the same manufacturing method as those used by the aforementioned coil component **10** (Sample No. 4), except that “Fe—Cr—Si alloy grains having a different  $d50$  (median diameter) value from that of the aforementioned coil component **10** (Sample No. 4) were used.”

As is evident from the volume resistivity and  $L \times I_{dc1}$  values of Sample Nos. 23 to 31, a volume resistivity higher than the aforementioned acceptance judgment criterion for volume resistivity ( $1.0 \times 10^7 \Omega \cdot \text{cm}$ ) can be obtained as long as  $d50$  is 20  $\mu\text{m}$  or less, while a  $L \times I_{dc1}$  higher than the aforementioned acceptance judgment criterion for  $L \times I_{dc1}$  ( $5.2 \mu\text{H} \cdot \text{A}$ ) can be obtained as long as  $d50$  is 3  $\mu\text{m}$  or more. In other words, excellent volume resistivity and  $L \times I_{dc1}$  can be obtained as long as  $d50$  (median diameter) is in a range of 3 to 20  $\mu\text{m}$ .

In essence, the above confirms that, as long as  $d50$  (median diameter) when the grain size is considered based on volume is in a range of 3.0 to 20.0  $\mu\text{m}$ , Fe—Cr—Si alloy grains whose  $d50$  (median diameter) is different can be used to achieve the same effects as mentioned above.

#### [Application to Other Coil Component]

Next, whether or not the ranges of values mentioned in the section “Verification of Optimal Granularity Distribution” and the section “Verification of Optimal Median Diameter” above can be applied (1) when the specific manufacturing method is different from the aforementioned coil component **10** (Sample No. 4), (2) when the type of coil component is the same but the specific structure is different from the aforementioned coil component **10** (Sample No. 4), (3) when grains different from the aforementioned coil component **10** (Sample No. 4) are used for the magnetic body **12**, and (4) when the type of coil component is different from the aforementioned coil component **10** (Sample No. 4), is explained.

(1) In the section “Example of Specific Method for Manufacturing Coil Component” above, the composition of magnetic paste was set to 85 percent by weight of Fe—Cr—Si alloy grains, 13 percent by weight of butyl carbitol (solvent) and 2 percent by weight of polyvinyl butyral (binder). However, the weights by percent of solvent and binder can be changed without presenting problems as long as the solvent and binder are removed in the binder removal process, to manufacture the same coil component as the aforementioned coil component **10** (Sample No. 4). The same applies to the composition of conductive paste.

Also, while butyl carbitol was used as the solvent for each paste, any other ether or even alcohol, ketone, ester, etc., can be used without presenting problems, instead of butyl carbitol, as long as it does not chemically react with Fe—Cr—Si alloy grains or Ag grains, and the same coil component as the aforementioned coil component **10** (Sample No. 4) can be manufactured using Pt grains or Pd grains instead of Ag grains.

In addition, while polyvinyl butyral was used as the binder for each paste, any other cellulose resin or even polyvinyl acetal resin, acrylic resin, etc., can be used without presenting problems, instead of polyvinyl butyral, as long as it does not chemically react with Fe—Cr—Si alloy grains or Ag grains, to manufacture the same coil component as the aforementioned coil component **10** (Sample No. 4).

Furthermore, the same coil component as the aforementioned coil component **10** (Sample No. 4) can be manufactured without presenting problems in particular, even when an appropriate amount of any dispersant, such as nonionic surface active agent or anionic surface active agent, is added to each paste.

Moreover, while the conditions of approx. 300° C. for approx. 1 hour were used for the binder removal process, other conditions can be set to manufacture the same coil component as the aforementioned coil component **10** (Sample No. 4), as long as the solvent and binder can be removed.

## 11

Also, while the conditions of approx. 750° C. for approx. 2 hours were used for the oxide film forming process, other conditions can be set to manufacture the same coil component as the aforementioned coil component **10** (Sample No. 4), as long as an oxide film of Fe—Cr—Si alloy grain can be formed on the surface of each grain and the properties of Fe—Cr—Si alloy grains do not change.

Furthermore, while the conditions of approx. 600° C. for approx. 1 hour were used for the baking process, other conditions can be set to manufacture the same coil component as the aforementioned coil component **10** (Sample No. 4), as long as the conductive paste can be baked without problems.

In essence, the ranges of values mentioned in the section “Verification of Optimal Granularity Distribution” and the section “Verification of Optimal Median Diameter” above can be applied even when the specific manufacturing method is different from the aforementioned coil component **10** (Sample No. 4).

(2) In the section “Example of Specific Structure of Coil Component” above, the magnetic body **12** had a length of approx. 3.2 mm, width of approx. 1.6 mm and thickness (height) of approx. 0.8 mm. However, the size of the magnetic body **12** has bearing only on the reference value of saturated magnetic flux density of the component itself, so effects equivalent to those mentioned in the section “Effects” above can be achieved even when the size of the magnetic body **12** is changed.

Also, while the coil **13** had approx. 3.5 windings, the number of windings of the coil **13** has bearing only on the reference value of inductance of the component itself, so effects equivalent to those mentioned in the section “Effects” above can be achieved even when the number of windings of the coil **13** is changed, and effects equivalent to those mentioned in the section “Effects” above can be achieved even when the dimensions or shapes of the segments CS1 to CS5 and IS1 to IS4 constituting the coil **13** are changed.

In essence, the ranges of values mentioned in the section “Verification of Optimal Granularity Distribution” and the section “Verification of Optimal Median Diameter” above can be applied even when the type of coil component is the same but the specific structure is different from the aforementioned coil component **10** (Sample No. 4).

(3) In the section “Example of Specific Structure of Coil Component” above, Fe—Cr—Si alloy grains were used to constitute the magnetic body **12**, but effects equivalent to those mentioned in the section “Effects” above can be achieved by using, for example, Fe—Si—Al alloy grains or Fe—Ni—Cr alloy grains instead, as long as the saturated magnetic flux density of the magnetic alloy grain material itself is higher than that of the conventional ferrite and an oxide film (=insulation film) is formed on the surface through heat treatment in an oxidizing ambience.

In essence, the ranges of values mentioned in the section “Verification of Optimal Granularity Distribution” and the section “Verification of Optimal Median Diameter” above can be applied even when magnetic alloy grains different from the aforementioned coil component **10** (Sample No. 4) are used for the magnetic body **12**.

(4) In the section “Example of Specific Structure of Coil Component” above, the coil component **10** was of the laminated type, but effects equivalent to those mentioned in the section “Effects” above can be achieved by adopting the present invention to a coil component of the powder-compacted type, for example, as long as the type of coil component is such that a helical coil is directly contacting a magnetic body. Here, a “coil component of the powder-

## 12

compacted type” refers to a coil component structured in such a way that a prepared helical coil wire is buried in a magnetic body made of magnetic powder using a press machine and, as long as Fe—Cr—Si alloy grains are used as the magnetic powder to constitute the magnetic body and the magnetic body is pressed and then heat-treated under the same conditions as those used in the aforementioned oxide film forming process, effects equivalent to those mentioned in the section “Effects” above can be achieved.

10 In essence, the ranges of values mentioned in the section “Verification of Optimal Granularity Distribution” and the section “Verification of Optimal Median Diameter” above can be applied even when the type of coil component is different from the aforementioned coil component **10** (Sample No. 4).

15 In the present disclosure where conditions and/or structures are not specified, a skilled artisan in the art can readily provide such conditions and/or structures, in view of the present disclosure, as a matter of routine experimentation.

20 Also, in the present disclosure including the examples described above, any ranges applied in some embodiments may include or exclude the lower and/or upper endpoints, and any values of variables indicated may refer to precise values or approximate values and include equivalents, and may refer to average, median, representative, majority, etc. in some embodiments.

25 The present application claims priority to Japanese Patent Application No. 2011-009886, filed Jan. 20, 2011 and Japanese Patent Application No. 2011-232371, filed Oct. 24, 2011, each disclosure of which is incorporated herein by reference in its entirety. In some embodiments, as the magnetic body, those disclosed in co-assigned U.S. patent application Ser. No. 13/092,381 (now U.S. Pat. No. 8,813,346) and Ser. No. 13/277,018 (now U.S. Pat. No. 8,723,634) 30 can be used, each disclosure of which is incorporated herein by reference in its entirety. Above U.S. Pat. No. 8,723,634 expressly states: “In some embodiments, by the oxidizing treatment, an oxide layer is formed on surfaces of the material grains by oxidizing Cr, Al, or the like (“another element”) which is an element constituting the material grains other than iron and which oxidizes more easily than iron, so that the oxide layer contains the other element in a quantity larger (e.g., 3 to 100 times higher, 5 to 10 times higher) than that in the material grains as shown in FIG. 5, 35 for example. In some embodiments, the material grains contain about 2% to about 8% by weight of Cr or Al (e.g., more than 3%). In some embodiments, the duration and the temperature of the oxidizing treatment are controlled so that the unprocessed grains aggregated via a binder can form an oxide layer thereon while partially sintering, i.e., performing partial grain growth, and also, the composition of the oxide layer can be controlled. As a result, in some embodiments, the grains are bonded with each other via the oxide layer and also via partial grain growth (some grains are partially fused (metal to metal bonding) with each other where the oxide layer is not formed while maintaining general shapes of the grains). The above can be observed by a SEM wherein some grains have cross-section outlines which can be fully observed as individual grains (each grain is fully covered with an oxide layer), and some grains have cross-section outlines which are connected to each other (grains are partially fused to each other, e.g., at least about 2/3 of the outline of individual grains are maintained), as illustrated in FIG. 1 of Japanese patent application No. 2011-222093, filed Oct. 6, 2011 (which claims priority to Japanese patent application No. 2011-100095, filed Apr. 27, 2011), the disclosure of which is herein incorporated by reference in its 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280

## 13

entirely. In some embodiments, the partially fused grains are connected, where no oxide layer or no other layer is formed, by, for example, metallic bonding where metal atoms of the grains are bonded together, by metal-to-metal connection where metal portions of the grains are contacted with each other without metallic bonding, and/or by bonding/connection partially using metallic bonding. In some embodiments, more non-fused grains than partially-fused grains may be observed, and in other embodiments, more partially-fused grains than non-fused grains may be observed, adjusting magnetic characteristics and volume resistance, for example, when a coil-type electronic component is constituted by the grains. The ratio of the number of fused grains to the total number of grains may be about 5% to about 80% (including 10%, 20%, 30%, 40%, 50%, 60%, 70%, and values between any the foregoing). Alternatively, substantially all grains are non-fused and have individual cross-section outlines.” U.S. Pat. No. 8,723,634 at column 16, line 48 to column 17, line 27.

It will be understood by those of skill in the art that numerous and various modifications can be made without departing from the spirit of the present invention. Therefore, it should be clearly understood that the forms of the present invention are illustrative only and are not intended to limit the scope of the present invention.

We claim:

1. A coil component of the type where a helical coil covered with a magnetic body is directly contacting the magnetic body, wherein the magnetic body is mainly constituted by magnetic alloy grains, other than ferrite grains, and is substantially free of a glass component, wherein the magnetic alloy grains consist of grains and an oxide of the magnetic alloy, said oxide being film covering the surface of the grains, said magnetic alloy grains being bonded together by the oxide film without any other binder and by metal-to-metal bonding of the grains made of the magnetic alloy where no oxide film is formed.

2. The coil component according to claim 1, wherein the oxide film of the magnetic alloy grains is formed on their surface through heat treatment in an oxidizing ambience.

3. The coil component according to claim 2, wherein the magnetic alloy grains are Fe—Cr—Si alloy grains.

4. The coil component according to claim 1, wherein when their grain size is considered based on volume, the magnetic alloy grains have their d10/d50 in a range of 0.1 to 0.7 and d90/d50 in a range of 1.4 to 5.0.

5. The coil component according to claim 2, wherein when their grain size is considered based on volume, the magnetic alloy grains have their d10/d50 in a range of 0.1 to 0.7 and d90/d50 in a range of 1.4 to 5.0.

6. The coil component according to claim 3, wherein when their grain size is considered based on volume, the magnetic alloy grains have their d10/d50 in a range of 0.1 to 0.7 and d90/d50 in a range of 1.4 to 5.0.

7. The coil component according to claim 1, wherein when their grain size is considered based on volume, the magnetic alloy grains have their d50 in a range of 3.0 to 20.0  $\mu\text{m}$ .

8. The coil component according to claim 2, wherein when their grain size is considered based on volume, the magnetic alloy grains have their d50 in a range of 3.0 to 20.0  $\mu\text{m}$ .

## 14

9. The coil component according to claim 3, wherein when their grain size is considered based on volume, the magnetic alloy grains have their d50 in a range of 3.0 to 20.0  $\mu\text{m}$ .

10. The coil component according to claim 4, wherein when their grain size is considered based on volume, the magnetic alloy grains have their d50 in a range of 3.0 to 20.0  $\mu\text{m}$ .

11. The coil component according to claim 5, wherein when their grain size is considered based on volume, the magnetic alloy grains have their d50 in a range of 3.0 to 20.0  $\mu\text{m}$ .

12. The coil component according to claim 6, wherein when their grain size is considered based on volume, the magnetic alloy grains have their d50 in a range of 3.0 to 20.0  $\mu\text{m}$ .

13. A coil component comprising:  
a magnetic body having a main structure constituted by magnetic alloy grains, other than ferrite grains, and being substantially free of a glass component, wherein the magnetic alloy grains consist of grains made of a magnetic alloy and an oxide of the magnetic alloy, said oxide being film covering the surface of the grains, said magnetic alloy grains being bonded together by the oxide film without any other binder and by metal-to-metal bonding of the grains made of the magnetic alloy where no oxide film is formed; and

a helical coil being in contact with and covered with the magnetic body, wherein a portion between the helical coil and magnetic alloy grains of the magnetic body adjacent to the helical coil is constituted by an oxide film formed between the helical coil and the adjacent magnetic alloy grains by oxidization of the adjacent magnetic alloy grains, and the adjacent magnetic alloy grains are bonded to the helical coil via the oxide film.

14. The coil component according to claim 13, wherein the helical coil is made of a sintered material of a conductive paste, said sintered material being formed when the oxide film is formed between the adjacent magnetic alloy grains and between the helical coil and the adjacent magnetic alloy grains.

15. The coil component according to claim 13, wherein the magnetic alloy grains are Fe—Cr—Si alloy grains.

16. The coil component according to claim 13, wherein the magnetic alloy grains have a size distribution such that d10/d50 is in a range of 0.1 to 0.7 and d90/d50 is in a range of 1.4 to 5.0, wherein d10, d50, and d90 represent the 10<sup>th</sup> percentile size, 50<sup>th</sup> percentile size, and 90<sup>th</sup> percentile size based on volume, respectively.

17. The coil component according to claim 13, wherein the magnetic alloy grains have their d50 in a range of 3.0 to 20.0  $\mu\text{m}$ , wherein d50 represents the 50<sup>th</sup> percentile size based on volume.

18. The coil component according to claim 1, wherein the magnetic alloy grains are also bonded by direct bonding of grains without the oxide film.

19. The coil component according to claim 1, magnetic alloy grains in the magnetic body near the helical coil are bonded to the helical coil by the oxide film without any other binder.

20. The coil component according to claim 13, wherein the adjacent magnetic alloy grains are bonded to the helical coil by the oxide film without any other binder.